

P. M. STEWART.

RIGID PIECE OF METAL INSULATED AGAINST ELECTROLYSIS AND CORROSION AND  
THE PROCESS OF MAKING THE SAME.

APPLICATION FILED SEPT. 16, 1912.

1,167,949.

Patented Jan. 11, 1916.

Fig.1.



Fig.2.



Witnesses:

M. G. Crozier,  
J. Murphy

Inventor,  
Perry M. Stewart  
by Jas. H. Lehigh  
Atty.

# UNITED STATES PATENT OFFICE.

PEREZ M. STEWART, OF NEW YORK, N. Y., ASSIGNOR OF ONE-HALF TO HAROLD H. ROBERTSON, OF SEWICKLEY, PENNSYLVANIA, AND ONE-HALF TO GERTRUDE F. STEWART.

## RIGID PIECE OF METAL INSULATED AGAINST ELECTROLYSIS AND CORROSION AND THE PROCESS OF MAKING THE SAME.

1,167,949.

Specification of Letters Patent. Patented Jan. 11, 1916.

Application filed September 16, 1912. Serial No. 720,492.

To all whom it may concern:

Be it known that I, PEREZ M. STEWART, a citizen of the United States, and a resident of the borough of Manhattan, city, county, 5 and State of New York, have invented an Improvement in Rigid Pieces of Metal Insulated Against Electrolysis and Corrosion and the Process of Making the Same, of which the following description, in connection with the accompanying drawings, is a 10 specification, like letters on the drawings representing like parts.

This invention relates to a novel process of insulating rigid pieces of metal against 15 electrolysis and corrosion and to the product of such process.

The process is especially applicable for treating large pieces of structural steel, such as beams, girders, etc., employed in the construction of buildings, bridges, and the like, whereby said steel structures are insulated and thereby protected against electrolysis and corrosion.

Prior to this invention many methods 25 have been devised and many compositions have been used for coating steel, with a view to absolutely excluding moisture, which it was well known, must be excluded in order to protect steel from electrolysis and 30 corrosion, but these methods and compositions have not been successful. No paint has as yet been devised which will absolutely accomplish this purpose. Linseed oil which is the vehicle for practically all paints designed for protective coatings, is recognized 35 by those skilled in the art to have several fatal defects. Even when the coat of linseed oil is skilfully applied, voids are bound to occur which will allow the entrance of 40 moisture to attack the coated surface. In order to avoid this objection, pigments have been used to fill these voids, but this method has been only partially successful. Gums have been added to make practically a varnish 45 coating, and while this has been fairly successful, the price is prohibitive, especially on large structures.

The slight amount of moisture or surface film which is found upon all steel structures, 50 unless heated beyond the boiling point of water, is sealed in by the paint in ordinary painting, thus leaving the film of moisture to continue its electrolytic action with the metal, producing rust underneath the paint.

The so-called protective coating of linseed oil in combination with many of the lead and zinc pigments is not a stable compound and after a comparatively short time a chemical change analogous to saponification takes place. It is therefore but a brief time before 55 moisture due to condensation removes the oily compound leaving the pigment, which, in itself, is not a protective coating, and is generally a rust promoter. This is the action commonly spoken of as "chalking". 60 One of the chief characteristics of pure linseed oil is the fact that it oxidizes, but it is not generally known that after this oxidation reaches a certain stage the compound thus produced is soluble in water. 65

Cushman and Gardner in their recent book on "*Corrosion and Preservation of Iron and Steel*" have this to say with regard to bituminous compounds: "From the standpoint of the electrolytic theory of corrosion, 70 it has repeatedly been stated in the foregoing pages that a natural insulator or non-conductor of electricity should be well adapted for the protection of iron. In view of the truth of this general principle, it 75 would seem that bituminous compounds were peculiarly well adapted for the purpose. Unfortunately, many materials which are well adapted for the protection of iron from one point of view are too prone to fail 80 from another. As a matter of fact, most bitumens will not stand free exposure to atmospheric conditions, water and sunlight. It is a significant fact that in the cases in which bitumens have been successfully used, 85 it has been under conditions in which the material was not, so to speak, normally exposed to sunlight and the atmosphere. To sum up the discussion of the use of bituminous paint and compounds as protective 90 coats for iron, the authors wish to reiterate their opinion that in special cases, and if properly selected, there are no better materials available". 95

In accordance with this invention, I have 100 provided a method for producing insulated structural steel shapes or members or any steel structure, no matter how large, in which the steel is insulated by a sheet or layer of asbestos paper against electrolysis 105 and corrosion and in which a bituminous composition is employed to secure the asbestos sheet or layer to the steel structure.

and is protected against the injurious action of sunlight, moisture and evaporation on such compounds by the sheet or layer of asbestos, as will be described, whereby the 5 bituminous composition remains in its original condition and effective as an adhesive for an indefinite length of time.

In accordance with the method employed by me, the steel structure is cleansed and heated, and while the steel is in a heated 20 condition, a layer or coating of fluxed asphalt is applied thereto, and almost immediately a sheet or layer of asbestos paper is applied to the asphalt layer, while the latter 25 is in an adhesive fluid condition. The asbestos sheet may then be coated with paint, cement, or layers of asphalt and felt or paper.

In the accompanying drawing I have 20 illustrated one form of protected structural steel member produced by my method and embodying my invention.

Figure 1 is a front view of an I column, and Fig. 2, a transverse detail sectional view 25 of the column shown in Fig. 1 on an enlarged scale.

In carrying out my process, the first step of cleaning the surface of the steel is preferably carried out when the structural shape 30 or member is at the job, in the field, or at the place of erection. All surfaces of the structural shape are first thoroughly cleaned and heated. The cleaning may be accomplished by wire brushing, sand blasting or 35 any other suitable mechanical or chemical method. The cleaning may also be accomplished by burning with one or more gasoline torches or any kind of suitable gas furnace. In any event the step of burning or heating 40 should be used, since this removes shop coat, oil, scale, surface film, moisture and other deleterious factors and at the same time heats the surface of the member, and opens the pores of the steel, rendering the 45 steel in a receptive condition to increase the adhesion and bond between the surface of the steel and the coating of bituminous composition which is next applied.

The bituminous composition should be applied 50 preferably immediately after burning and while the metal is still heated, and may be applied either hot or cold but preferably hot.

The bituminous composition for the best 55 results is a fluxed bitumen, that is, a high grade asphalt having a high melting point, namely about 225° to 250° F., is tempered or fluxed by the addition of animal fats or slow drying oils, such as stearin pitch in 60 the proportion of from 5 to 10%, which flux has the effect of making the bitumen more durable, tenacious, pliable, and of retaining its elasticity for a long time. While the coating of the bituminous composition is 65 still soft, a layer or sheet of asbestos paper

is applied with pressure to the coated surface of the metal structure, and this process is repeated until the whole of one surface of the rigid steel member is covered by the 70 layer of bituminous composition and the 75 layer or sheet of asbestos paper, which is especially serviceable for the purpose, for the following reasons: (1) The sheet of asbestos is not penetrated by the actinic rays of the sun, which have a deleterious effect 80 on the asphalt, in that they take the life out of the asphalt and render it liable to crack and expose the steel. (2) The sheet of asbestos normally contains from seven to fourteen per cent. of water of its own, that is, by absorption, and in addition about four per cent. of water of crystallization, and therefore the asphalt coating is practically 85 protected by a wall of water in the asbestos sheet, which prevents the oil in the asphalt 90 from passing through the asbestos sheet and therefore prevents evaporation of the oil and the deterioration of the asphalt coating, which remains unchanged for an indefinite 95 length of time.

The asbestos sheet or layer may be painted or otherwise treated on its exposed surface to waterproof it, or it may have applied to it additional layers of bituminous composition and asbestos, felt, paper or cement. 95 It is preferred to protect the layer or sheet of asbestos with paint or other material as described, but it is not desired to limit the invention in this respect as good results 100 would be obtained with the plain asbestos sheet alone.

In the present instance, the I column shown in the drawing is provided with a plurality of layers of bituminous composition and asbestos.

In Fig. 2, A represents the first layer of bituminous composition, B the layer of asbestos paper, C a layer of bituminous composition on the layer B, D a layer of asbestos paper, E a layer of bituminous composition applied to the layer D, F a layer of waterproof fabric in the form of prepared felt, muslin or linen, G a layer of bituminous composition or mastic. The protected I column may be embedded in concrete or other 115 suitable fireproof building material J.

In some instances it may be desirable to provide the steel structure with a plurality of layers of bituminous composition and sheets or layers of asbestos, but in most cases, 120 it will be sufficient to provide a single layer of bituminous composition and a single sheet or layer of asbestos, and render the latter waterproof by painting the exterior surface thereof, for in the simpler construction it will be seen that the steel member is thoroughly 125 protected against electrolysis and corrosion, by the layer of the bituminous composition and by the sheet of asbestos, for the reasons above set forth and further by the additional 130

layer of paint or other waterproof material, which prevents evaporation of the water wall in the asbestos layer, and also prevents moisture penetrating into the asbestos.

5 In some cases, as for instance in buildings, it may be preferred to protect all the surfaces of the steel structure or member, whereas in the same and other structures, such for instance as bridges and the like, 10 it may be found sufficient to protect only those surfaces of the steel member which are exposed to the atmosphere. In either case, the surface of the steel member covered by the bituminous composition and the sheet 15 or layer of asbestos is thoroughly protected from the deleterious action of extraneous fumes, gases, atmospheric conditions and stray or ground electric currents, and also from interior deterioration, that is, deterioration of the bituminous composition.

Claims:

1. The process of insulating structural steel shapes to prevent electrolysis and corrosion, which consists in cleaning and heating the surfaces of the steel structure to remove scale, dirt, moisture, etc., and to open the pores of the steel, applying to the steel structure thus cleaned and while in a heated condition a fluxed bituminous composition, 25 applying to said coating of bituminous composition while the latter is soft a layer of asbestos paper in its normal condition, and applying to the exterior surface of the asbestos paper a waterproof coating, for the 30 purpose specified.

2. The process of insulating structural steel shapes to prevent electrolysis and corrosion, which consists in cleaning and heating the surfaces of the steel structure to remove scale, dirt, moisture, etc., and to open the pores of the steel, applying to the steel structure thus cleaned and while in a heated condition a fluxed bituminous composition, 40 and applying to said coating of bituminous composition while the latter is soft a layer of asbestos paper in its normal condition.

3. The process of insulating a rigid piece of metal, which consists in heating the outer 50 surface of the metal piece to expel moisture and open the pores of the metal, covering the said surface while in a heated condition with a layer of bituminous composition, and applying to the bituminous layer while soft a sheet of insulating material which is impervious to sunlight and in its normal condition.

4. As an improved article of manufacture, 60 a rigid piece of corrodible metal having its outer surface free from deleterious substances protected by a layer of bituminous composition applied to the said surface, and penetrating into the pores thereof, and a

layer of asbestos paper adhesively secured to the rigid metal structure by said bituminous coating which penetrates one surface 65 of the asbestos layer, substantially as described.

5. The process of insulating a rigid piece of metal, which consists in cleaning the rigid 70 article, coating the rigid article thus treated with a layer of bituminous composition, applying to the bituminous layer while soft a layer of asbestos, folding the layer of asbestos about the coated rigid article to envelop 75 the same, and pressing the asbestos layer into firm contact with the rigid article.

6. The process of insulating a rigid piece of metal, which consists in cleaning the rigid 80 article, coating the rigid article thus cleaned while in a heated condition with adhesive material, applying to the metal article thus coated and while the coating of adhesive material is soft, a layer of fibrous insulating material, folding the layer of fibrous insulating material about the coated rigid article 85 to envelop the same, and pressing the fibrous insulating layer into firm contact with the rigid article.

7. As an improved article of manufacture, 90 a rigid piece of corrodible metal having its outer surfaces free from scale, dirt, oil and moisture and protected by a layer of bituminous composition applied to the said surfaces and penetrating into the pores thereof, 95 and a layer of asbestos paper enveloping said rigid metal structure and adhesively secured thereto by said bituminous coating which penetrates one surface of the asbestos layer.

8. As an improved article of manufacture, 100 a rigid piece of corrodible metal having its outer surfaces free from scale, dirt, oil and moisture and protected by a layer of bituminous composition applied to the said surfaces and penetrating into the pores thereof, 105 and a layer of fibrous insulating material enveloping said rigid metal structure and adhesively secured thereto by said bituminous coating.

9. As an improved article of manufacture, 110 a rigid piece of corrodible metal having its outer surfaces free from deleterious substances and protected by a layer of adhesive material applied to said surfaces, and a layer 115 of fibrous insulating material enveloping said rigid structure and secured thereto by said adhesive coating.

In testimony whereof, I have signed my name to this specification in the presence of 120 two subscribing witnesses.

PEREZ M. STEWART.

Witnesses:

LEWIS C. KUDEGEL,  
HAROLD R. ZEAMANS.